

## UNITED STATES PATENT OFFICE

2,136,655

## BEARING ALLOY

Julian G. Ryan, Wood River, Ill., assignor to  
Shell Development Company, San Francisco,  
Calif., a corporation of Delaware

No Drawing. Original application October 18,  
1937, Serial No. 169,645. Divided and this ap-  
plication March 26, 1938, Serial No. 198,271

3 Claims. (Cl. 75—151)

This invention is chiefly concerned with bearing compositions used in internal combustion engines. It has been recognized that bearings should comprise at least two constituent parts, 5 namely, a soft part to conform to the crankshaft and readjust itself to irregularities in operation and a hard part to support the load and have anti-frictional qualities in order not to seize onto the shaft. These properties have in the past been 10 found in tin base bearing alloys commonly known as "babbitt".

This application is a division of my application Serial No. 169,645 filed October 18, 1937.

In recent years owing to the greater speeds required of automotive engines, the higher oil temperatures produced have caused a softening of the babbitt and in some cases, actual melting due to the eutectic melting point being around 450° F. and the softening point being around 20 212° F.

Endeavor has therefore been made to develop bearing metals which would have anti-friction properties and have a high enough melting point that the softening temperature would be raised 25 above that of the tin base bearings and at the same time be economical.

Two of the bearing materials which have been produced to meet this requirement are cadmium-silver and cadmium-silver-copper compositions. 30 Cadmium is the main constituent of these compositions. Cadmium has a melting point of about 650° F. and a Brinell hardness of over 20. Furthermore cadmium has good bonding properties as evidenced by its successful use with zinc in 35 high strength solders.

Silver, when added to the cadmium in relatively small quantities, improves the casting qualities of cadmium by making it less susceptible to oxidation at casting temperatures and by increasing 40 the fluidity. Silver, further, has a marked influence upon the physical characteristics of cadmium by improving grain structure.

A typical cadmium silver bearing alloy will have the following composition: cadmium 97.75% 45 and silver 2.25%, the silver being held in solution by the cadmium.

The addition of small amounts of copper to the composition has the property of raising the Brinell hardness appreciably. A typical cadmium-silver-copper composition is as follows: cadmium 50 98.75%, silver 0.75% and copper 0.50%.

These bearings have, in general, been quite successful. However, in many cases, corrosion of the bearing has taken place. Many theories have 55 been advanced to explain this, and various oil

compositions have been devised to reduce this corrosion in the belief that it was entirely due to the lubricant used. However, I have discovered that one of the main causes of becoming corrosive can be traced to the composition of the bearing alloys, and it is the object of this invention to provide substantially non-corrosive bearings for 5 internal combustion engines.

I have found that the corrosion is in part due to galvanic action between the constituents of the 10 bearing material submerged in mineral or hydrocarbon oil. This galvanic action takes place through the intermediary of the lubricating oil. The electrical conductivity of the oil is very slight under normal circumstances, but upon oxidation 15 of the lubricant and the accumulation of small amounts of water in the crankcase of the motor the conductivity is materially increased.

According to my investigation, I have found that in some cases the cadmium-silver bearings 20 after being run in an automobile motor for several hours showed pitting of the bearings. Subsequent analysis of the oil failed to show any cadmium particles in the oil, thus eliminating abrasion of the metal or insufficient oiliness of 25 the oil as the cause of corrosion. This led to the conclusion that at least part of the corrosion was due to electrochemical action. This conclusion was further supported by the fact that only the cadmium went into solution and silver was not 30 found dissolved in oil in conformity with its lower position in the electromotive series. Further experiments were then conducted to establish the electrode potentials between cadmium and silver 35 electrodes placed in a used motor lubricating oil bath. Measured at an oil temperature of 210° F. a potential of .630 volt was established. In order to investigate the effect of electrolyte further, small buttons of polished cadmium with pure silver inserts were exposed to oils under a 40 variety of test conditions. The polished surface was examined under a microscope before and after the tests. The results of these tests showed that cadmium corrodes easily and that galvanic 45 action accelerates the corrosion. The silver inserts were not attacked. A series of tests with numerous alloys have established that there exists a direct relationship between the rate of corrosion of an alloy and the electric potential between the electrodes made of the alloyed metals, when 50 these electrodes are placed in a lubricating oil electrolyte.

I have found that by alloying a small quantity of a potential depressing substance with the bearing material corrosion may be prevented or 55

at least substantially reduced. Of various substances tested in alloys with the cadmium-silver and cadmium-silver-copper bearings I have found that antimony is particularly effective for the purpose desired.

Below are tabulated the results obtained using an oil electrolyte at 340° F.

| 10 | Composition of cathode | Composition of anode             | Equilibrium potential millivolts |
|----|------------------------|----------------------------------|----------------------------------|
|    | Silver.....            | Cadmium.....                     | 545                              |
|    | Do.....                | Cadmium+0.2% antimony by wt..... | 470                              |
|    | Do.....                | Cadmium+2.0% antimony by wt..... | 410                              |
| 15 | Do.....                | Cadmium+5.0% antimony by wt..... | 395                              |

From the above it will be seen that cadmium alone gave an equilibrium potential of 545 millivolts. Corrosion of the cadmium was apparent after about 15 minutes in the test cell. During this time the surface of the cadmium electrode changed considerably. At first it had a bright polished finish but later showed a coarse grain structure. The addition of antimony to cadmium reduced the potential and corrosion with the result that the cadmium-antimony electrodes after an hour, had a very fine grained finish and showed only slight corrosion. Microscopic examination showed that the crystal structure of the metal was changed by the presence of the antimony. This is probably also a factor in reducing corrosion.

Further tests were made, using a silver cathode and an anode of standard cadmium-silver-copper bearing metal and anodes of the same with small amounts of antimony added. The results of these tests are tabulated below using the same oil at 340° F.

| 40 | Composition of cathode | Composition of anode                                          | Equilibrium potential millivolts |
|----|------------------------|---------------------------------------------------------------|----------------------------------|
|    | Silver.....            | Commercial cadmium-silver-copper.....                         | 525                              |
|    | Do.....                | Commercial cadmium-silver-copper+0.1% antimony by weight..... | 495                              |
| 45 | Do.....                | Commercial cadmium-silver-copper+0.2% antimony by weight..... | 465                              |

To obtain further information regarding the addition of antimony to bearing alloys the fol-

lowing test was made: Small pieces of the same material as was used for the anodes in the above test were machined into the form of cylindrical slugs weighing 8 grams each, carefully polished and washed with solvent. Each specimen was then placed in a test tube containing a measured amount of a used lubricating oil. The test tubes and contents were each kept at a temperature of 340° F., air was continually bubbled through the oil to simulate actual operating conditions. At the end of a period of sixteen hours the slugs were removed and after careful washing and drying, were weighed. The results are shown below:

| 15                                       | Alloy | Number of specimens | Average loss |
|------------------------------------------|-------|---------------------|--------------|
|                                          |       | Mgs.                |              |
| 1. Commercial cadmium-silver-copper..... | 9     | 24                  | 20           |
| 2. (1)+0.1% antimony.....                | 5     | 13                  |              |
| 3. (1)+0.2% antimony.....                | 5     | 7                   |              |

From the above it appears conclusively that both by equilibrium potential tests and actual corrosion tests of the bearing metal that antimony has the effect of reducing the corrosion of bearing when added in small quantities. Antimony hardens the alloy and for this purpose copper has been in the past added to cadmium-silver bearings. It is therefore possible to replace the copper with antimony which will serve both to harden the alloy and reduce corrosion.

While I have shown only tests using specific amounts of antimony, the conclusion must be drawn that amounts between the examples will be beneficial for the purpose intended and that I do not intend to limit myself to the exact proportions given.

I claim as my invention:

1. A bearing metal consisting of silver 0.5% to 1%, copper 0.25% to 0.75%, antimony 0.1% to 1% and the remainder cadmium.
2. A bearing metal consisting of silver 0.5% to 1%, copper 0.25% to 0.75%, antimony 0.1% to 0.2% and the remainder cadmium.
3. A bearing metal consisting of silver 0.5% to 1%, copper 0.25% to 0.75%, antimony 0.1% and the remainder cadmium.

JULIAN G. RYAN.